

July 7, 1959

F. X. McCAWLEY

2,893,115

METHOD OF COATING AND WORKING METAL

Filed June 28, 1957



INVENTOR

FRANK X. McCAWLEY

BY

*Reginald S. Dean*

ATTORNEY

1

2,893,115

## METHOD OF COATING AND WORKING METAL

Frank X. McCawley, Cheverly, Md., assignor to Chicago Development Corporation, Riverdale, Md., a corporation of Delaware

Application June 28, 1957, Serial No. 668,771

1 Claim. (Cl. 29—424)

This invention relates to titanium carbide coatings on metals and methods for their production. I have found that thin adherent layers of titanium carbide provide the most effective barrier layers to prevent the penetration of gases and the diffusion of other metallic materials into steel, titanium and other metals.

I have found such layers particularly useful in protecting titanium and titanium alloys from contamination during hot working. The carbide layer remains intact during rolling and penetrates into the metal to only a very small depth.

I prefer to produce the titanium carbide layer by an electrolytic process. For this purpose, I provide a molten bath of strontium, barium, sodium, potassium, lithium or calcium chloride. The bath may contain a mixture of these chlorides. I prefer a mixture of alkaline earth and alkali chlorides. I particularly prefer to use a bath containing 65%  $\text{SrCl}_2$ , 35%  $\text{NaCl}$ , because such a bath is molten at relatively low temperatures and 8-10% titanium can be dissolved in it as lower chlorides together with one of the alkali or alkaline earth metals.

When the metal to be coated with TiC is coated with graphite and made a cathode in such a bath, a layer of titanium carbide is formed on its surface. The thickness of this layer depends on the thickness of the adherent graphite layer which can be applied. In most cases, this is on the order of 1 mil.

The extent of protection afforded for a titanium surface during hot working is illustrated in the sole figure which shows the oxygen penetration for unprotected titanium, for titanium protected by a salt layer and for titanium protected by a layer of titanium carbide.

I have used other procedures for producing a layer of titanium carbide on titanium such as heating to a high temperature in argon containing a small percentage of hydrocarbon gas. I have found, however, that titanium carbide layers produced in this manner are less adherent and protective.

Having now described my invention in its more general terms, I will illustrate it by examples.

### Example I

I take an ingot 4" x 4" x 10" of titanium-vanadium alloy containing 4% V, .01% oxygen, balance substantially titanium. I split this lengthwise to obtain two identical portions each 2" x 4" x 10". I coat one of these with graphite and make it a cathode in a cell having a particulate titanium anode contained in an annular perforate iron basket and the cathode disposed in the center of the cell surrounded by the perforate basket. The cell is provided with an inert atmosphere and means for raising the cathode out of the bath and cooling it in an inert atmosphere. The cell bath consisted of 65% strontium chloride 35% sodium chloride in which was dissolved 8% titanium as chloride, average valence 2.4 and 3% alkalinous metal calculated as sodium. A di-

2

rect current of 15 amperes was passed for 20 minutes at 750° C.

After cooling in an inert atmosphere, the portion of the ingot with adhering salt, fine titanium crystals and titanium carbide layer is placed in a furnace at 900° C. along with the untreated portion. Heating is continued for 1 hour and both pieces are hot rolled to 1/2" thickness without reheating. They are then reheated for 15 minutes and hot rolled to 1/4" thickness. Both pieces are then scalped to remove 4 mils of the original metal on both sides. The piece protected by the plating operation then analyzed .014 oxygen and the other piece .071 oxygen.

### Example II

I take a bar 1/4" x 12" x 3' steel and treat it in the same manner as the titanium alloy ingot in Example I to produce a coating of titanium carbide on the bar. I hot roll this bar at 750° C. to 40 gauge strip. The resulting strip has a coating of titanium carbide which protects the steel from surface contamination. I take several portions of the sheet and galvanize it by hot dipping. The adherence of the zinc is good and the brittle layer of iron zinc alloy common in hot galvanizing is absent.

### Example III

I proceed as in Example I except that the cell bath is  $\text{NaCl}$  in which is dissolved 4.5% titanium as chloride, average valence 2.4 and .3% sodium. The bath temperature is 850° C. The metal treated is highly pure zirconium. The results are identical with those of Example I.

### Example IV

I proceed as in Example I except that I use a cell bath of 90%  $\text{KCl}$  10%  $\text{BaCl}_2$  in which is dissolved 2% titanium as chloride, valence 2.15 and 2.5% alkalinous metal (calculated as K). The metal to be treated is a zirconium alloy containing .2% iron. The results as to oxygen absorption on hot rolling are the same as in Example I.

### Example V

I proceed as in Example I except that the cell bath is 50%  $\text{CaCl}_2$  50%  $\text{LiCl}$  and the metal to be treated is pure titanium. The temperature of the cell bath is 800° C. The results obtained are identical with those in Example I.

### Example VI

I take a strip 1/4" thick of pure titanium containing .01% oxygen and substantially no other impurities. I heat this strip in a mixture of  $\text{CH}_4$  and  $\text{TiCl}_4$  at 800° C. whereby to coat it with TiC. I hot roll the so-coated strip at 850° C. to reduce it to one-half its thickness. I scalp .004 inch from each side. The resulting strip analyzes .02% oxygen.

### Example VII

In this example I apply the procedure of my invention to the protection of titanium-aluminum alloys during hot working. Such alloys of usual purity containing 10% aluminum have been found to break up when hot rolled at 1650° F. I have found that this is due to very rapid oxygen absorption. In this example I make an ingot of aluminum-titanium alloy containing 10% aluminum, .02% oxygen, and substantially no other impurity. I cast this ingot by rubbing with flake graphite and then provide a further carbon coating by exposing the ingot to a smoky acetylene flame. I make this ingot a cathode in a bath consisting of calcium chloride having dissolved therein 10% titanium chloride, average valence 2.4, and 3% metallic calcium, the anode is particulate titanium. I employ a cathode current density of 100 amperes/sq.

ft. for 15 minutes. A titanium carbide layer is formed on the ingot which layer is covered with salt and finely divided titanium. The so protected ingot is heated to 1650° F. in air and hot rolled. The hot rolling proceeds smoothly, and an analysis of the hot rolled bar after removing .005 inch from the surface shows 10.1% aluminum, .025% oxygen, balance substantially titanium.

What is claimed is:

The method of fabricating a metal selected from the group consisting of titanium, and zirconium, and alloys consisting principally of these metals which consists in coating said metal with carbon and making it a cathode in an electrolytic cell having a fused electrolyte of at least one chloride selected from the group consisting of calcium, strontium, barium, sodium, potassium and lithium chlorides and dissolved therein 1-10% titanium as lower

10

5

chlorides and .1-5% of a metal corresponding to the chlorides of the fused electrolyte, and passing a direct current from a particulate titanium anode to said cathode whereby to form a coating on the cathode surface and then fabricating the metal by subjecting it to working at temperatures from 750-900° C., whereby to limit oxygen absorption to .02% when a surface layer about 5 mils thick is removed.

#### References Cited in the file of this patent

#### UNITED STATES PATENTS

|           |                 |                |
|-----------|-----------------|----------------|
| 2,686,355 | Lundin et al.   | Aug. 17, 1954  |
| 2,786,809 | Raynes          | Mar. 26, 1957  |
| 2,797,476 | Sendzimir       | July 2, 1957   |
| 2,807,575 | Charlton et al. | Sept. 24, 1957 |